

[54] PROCESS FOR CASTING MOLTEN METAL

[75] Inventors: William A. Pavlo, Fleetwood, Pa.;  
Richard M. Conroy, Dallas, Tex.[73] Assignee: General Battery Corporation,  
Reading, Pa.

[22] Filed: Sept. 29, 1972

[21] Appl. No.: 293,461

[52] U.S. Cl. .... 164/65, 164/133, 164/337,  
164/338

[51] Int. Cl. .... B22d 27/16

[58] Field of Search .... 164/65, 66, 68, 133, 256,  
164/258, 259, 335, 337, 338 H

## [56] References Cited

## UNITED STATES PATENTS

2,060,134 11/1936 Summey .... 164/259 X

3,467,167 9/1969 Mahin ..... 164/66 X

Primary Examiner—Robert D. Baldwin

Assistant Examiner—John E. Roethel

Attorney, Agent, or Firm—Paul &amp; Paul

## [57] ABSTRACT

It is herein provided to mold castings of articles, such as battery grids, in accordance with a technique for permitting the molten metal to have a higher lead content, by raising the temperature of the melt at the point of molding, or substantially thereto, but not significantly prior thereto. Accordingly, the metal is initially heated to a desired liquid conveying temperature, and, on its path of delivery to a ladle, from which it will be poured for casting, the melt is superheated, or boosted up to the desired temperature, either in a single stage, or in two stages.

9 Claims, 1 Drawing Figure



PATENTED JUN 11 1974

3,815,659



## PROCESS FOR CASTING MOLTEN METAL

## BACKGROUND OF THE INVENTION

In the battery industry, and most particularly, in that portion of the industry directed to satisfying the demands of the automotive industry, it has become commonplace, in response to the demands of the automobile industry, to provide batteries having immediate or substantially immediate high terminal voltage, for facilitating the provision of increased cranking power, or to provide the voltage (generally 6 volts or 12 volts) at an increased amperage, in order to effectively crank high compression engines, or engines having larger displacement.

In the batteries available for use by the automotive industry, namely lead acid batteries, reliance is made upon the ability of the plate surface to hold a charge, at a potential relative to other plates. Accordingly, a great number of surface charges, induced by surface voltage, aggregatively provide the cranking power. The greater the available plate surface, the more power that may be provided by a battery. One answer to this problem is to construct larger batteries, in order to facilitate the provision of battery plates or grids having increased surface area. However, with the trend toward size standardization of components, such as batteries, for interchangeability with different models of cars, irrespective of the amount of cranking power needed or the like, as well as with the tendency toward economizing available space, it has become impractical, to increase the size of batteries as an answer to this problem.

Another answer to the problem would be to increase the number of plates in each cell. To do so would require the construction of battery grids that are substantially thinner than those presently being utilized, in order to permit the total surface area to be substantially increased. However, due to problems inherent in the casting of metal, and due to limitations in available casting equipment itself, it is impractical to satisfactorily produce battery grids that are as thin as would be required.

Even with conventional casting equipment, in order to keep the melt at a sufficiently fluid level, having a desirably low level of surface tension, an alloy is used in the melt, that contains not only lead, but a significant percentage of antimony. However, the presence of antimony in the battery shortens the battery shelf life, and produces more maintenance problems with the battery than would be the case, if the battery were constructed of an antimony-free melt.

It is thus seen that for purposes of construction of battery grids, it has become commonplace to utilize antimony in the melt, such antimony being provided at significant percentages, depending upon the pouring, fluid-flow situation of the melt that is desired, etc. However, it would be preferable not to use significant amounts of antimony in the melt, for the above-mentioned reason.

It has been found that it is possible to reduce the level of antimony in the melt, and to compensate therefor during the casting process, by increasing the casting temperature, in order that the surface tension of the alloy will be sufficiently low to make good castings, even with alloy of low antimony content. However, at such higher temperatures, induced at the supply pot and carried through the piping from the pot to the la-

dle, such would induce excessive oxidation and drossing, or the formation of a scum on the surface of the melt, would be the result, thereby causing casting imperfections.

## THE PRESENT INVENTION

The present invention is directed toward providing a system whereby low antimony content of the melt may be used, but wherein a high casting temperature is employed, but wherein such high casting temperature is not applied until the last possible moment, prior to casting itself. This is done by first raising the temperature at the pot to a level that is sufficiently high in order to facilitate conveyance (as by pumping) throughout the delivery line, but which is sufficiently low that only insignificant amounts of oxidation will occur in the melt. Then, the temperature of the melt is raised just prior to casting, preferably in a subsequent two-stage operation, of first raising the temperature just prior to delivery of the melt to a ladle, preferably in an oxygen-free (or substantially free) atmosphere for further reducing the potential toward oxidation, such boost in temperature being preferably to a level just below what would be a good casting temperature for the metal, followed by another boost in temperature of the metal at the ladle itself, prior to pouring the metal from the ladle, into the mold.

## SUMMARY OF THE INVENTION

In accordance with the present invention, the temperature of the melt is substantially increased after the melt has left the supply pot, and prior to ladling the melt into a mold, in order to minimize opportunity for oxidation of the melt, such increase preferably being accomplished in a superheater located just prior to the ladle, for raising the temperature of the melt delivered to the ladle.

Accordingly, it is a primary object of this invention to provide novel casting method and apparatus.

It is a further object of this invention to provide a novel technique for the formation of battery grids.

It is another object of this invention to provide a novel molding technique, for molding castings having a high lead content.

It is another object of this invention to provide novel method and apparatus for making battery grids having reduced antimony content, wherein a superheater is utilized for raising the temperature of the melt subsequent to the application of heat to the melt in the melting pot.

It is a further object of this invention to accomplish the above object, wherein the step of raising the temperature occurs as part of a two-stage operation, with the temperature first being raised in a superheater, to a level just below that of the desired casting temperature, and with the temperature then being raised in the ladle itself, to the desired casting temperature.

Other objects and advantages of the present invention will become readily apparent to those skilled in the art from a reading of the following brief description of the drawing FIGURE, detailed description of the preferred embodiment, and the appended claims.

## IN THE DRAWING

The FIGURE is a schematic view of an apparatus embodying the system of this invention, and which is adapted for performing the method of this invention.

DESCRIPTION OF THE PREFERRED  
EMBODIMENT

Referring now to the FIGURE, it will be seen that a pot 20 is provided, for receiving lead, and a small amount of antimony 21 therein, by a suitable chute 22 or the like, with the material (lead and antimony) being in pellet form or the like, if desired, and with the pot 20 being provided with a gas burner or the like 23, for heating metal within the pot to a desired temperature. The burner 23 is of the open flame type, and may be provided with a fuel and air mixture for combustion or the like through a delivery line therefor 24, from any suitable source, with a control valve 25 being provided in the line 24, for a purpose which will be discussed hereinafter.

The temperature of the melt formed in the pot 20 will generally be about 700° Fahrenheit, which is significantly lower than the temperature for melt in pots utilized in accordance with conventional battery grid casting techniques. In any event, the temperature of the melt in the pot 20 will be brought to a sufficient level to permit fluid or "liquid" delivery therefrom, by means of a suitable molten metal pump 26 or the like, or by any other conventional means, through a line 27, whereby the melt will be delivered to the inlet 28 at the lower end of a superheater 30.

The superheater 30 is provided with a pair of gas burners 31 and 32, constructed of conventional manifold-burner arrangement, each to have a plurality of burner jets of the open flame type supplied by a suitable fuel-air or fuel-oxygen source or the like, as desired, from a suitable delivery line 33, and with a control valve 34 being disposed at the inlet of the connected-together manifolds, 31, 32. It will be apparent that, at a temperature of about 700°, even a low antimony-content lead melt in the pot 20, will not significantly oxidize.

In the superheater 30 (which is closed except for its inlet and outlet, in order to facilitate a substantially controlled oxygen atmosphere for the heating of melt disposed therein), the melt is raised to a temperature that may be approximately 1,000° F., but which will generally be within, but about 10° F. less than the desired casting temperature of the melt. The superheater 30 is generally cylindrical in configuration, and is provided with an outlet 35, at a higher level in elevation than the inlet 28, in order to facilitate the passage of the hot melt at an upper level within the superheater 30, first outwardly of the superheater 30, past a metering valve 36 or the like, for discharge from the line 37, to the ladle 38. It will be noted that the metering valve 36 may optionally be provided in the outlet line 35, but, if utilized, may facilitate the provision of a metered quantity only to the ladle 38, returning any excess back to the pot 20 through the line 40, thereby preventing the wasting of melt, as well as preventing the inefficient waste of energy utilized to raise such excess melt to the desired temperature.

The ladle 38 may be of trough-like construction as illustrated, and may be pivotable about the point 41, upon actuation of a valve 42 in fluid line 43, which would control a piston cylinder 44, for actuation of a piston therein, for tilting of the trough 38 in the direction of the arrow 45 illustrated in the drawing, when it is desired to pour the melt from the trough 38. However, it will be understood that any suitable or conven-

tional means may be utilized to discharge the melt from the ladle or trough 38.

It will be noted that a manifold 46 having a plurality of open-flame burners is provided, for heating the melt within the ladle 38, just at the point or stage in the process that the melt is adapted for pouring into a mold 47, with the heating device 46 being supplied with a fuel-air, or fuel-oxygen supply from a suitable source, through a supply line 48 therein, for controlling the amount of heat supplied to the ladle 38.

It will be seen that a pyrometer, pyrotroller or the like 50, may be utilized to control the amount of heat delivered to the manifolds 31, 32 of the superheater 30, by controlling the fuel-air (or oxygen) supply thereto, by control of the valve 34, from the line 51, and with the meter or control device 50 being operated in response to the temperature sensed by a thermocouple 52 or the like disposed directly in the melt within the superheater 30, and connected to the device 50 by a wire 53 of conventional type.

Also, the metering valve 36 may be controlled by the device 50, if desired, to open at the time that the temperature within the superheater 30 reaches a desired predetermined level. In the alternative, the metering device 36 could be controlled manually, or by a timing device or the like, if desired, or eliminated altogether, and with the metering being provided by the control of the pump 26, or even by the delivery of material into the pot 20, if desired.

Similarly, another pyrometer, pyrotroller or the like 55 is provided, actuated by a thermocouple 56 disposed for contact with the melt within the ladle 38, in order to control the temperature applied to the ladle 38 by the burners on the manifold 46, by controlling the amount of fuel and/or air or oxygen, delivered through the line 47, past the valve 48, by control of the valve 48.

Also, similarly a pyrotroller, pyrometer 57 or the like actuated by a thermocouple 58 disposed within the pot 20, may control the valve 25, for controlling the fuel supplied for raising the temperature of the melt within the pot 20, only to a desired level for reasons aforesaid.

It will be apparent that the various controls 50, 55 and 57 may be controlled in any given sequence, or programmed by a computer or the like 60, or other suitable control device 60.

Also, the overall control device 60 may also control the operation of the valve 42, by a suitable line connection 61 or the like thereto, for timing or otherwise controlling the ejection of melt from the ladle 38, by timed actuation of the piston cylinder 44, or of any other suitable discharge means.

It will also be apparent, that, if desired, the temperature of the melt within the superheater 30 may be raised in a single stage (eliminating use of the manifold and burner arrangement 46), such that once the melt was delivered to the ladle 38, it could be ladled therefrom, into the casting mold 47, without further increase in temperature. In that event, the temperature of the melt would be raised by the superheater 30, to at least (or above) the desired pouring temperature. However, in the preferred arrangement, and in the preferred utilization of this invention, the temperature increase will take effect in two stages, the first being in the superheater, to within about 10° of pouring temperature, with the latter 10° increase occurring while the melt is

within the ladle 38, immediately prior to pouring therefrom.

The apparatus and process of this invention makes a significant step toward eliminating the burning of antimony in the lead pot 20 that also causes drossing, by the use of a lead pot 20 that is kept at a temperature significantly below that of prior art types.

A further advantage of this invention, is in a saving that is effected in the alloy, in that, by the significant reduction of drossing, a substantial weight of the alloy is usable, and does not form a scum which would have to be removed unless contamination were tolerable. A significant factor in this elimination or reduction of drossing is that the alloy is raised a significant amount, and at a significant level (about 300° to 400°) in a controlled oxygen atmosphere (which means oxygen-free or substantially oxygen-free) within the superheater 30, in that the superheater 30 is closed to air (and oxygen) intermediate its ends except for the inlet 28 and discharge 35 thereof and any oxygen initially present therein will be driven off during an early heating stage thereof.

The mold 47, after discharge of the melt thereinto, may then be delivered along a conveyor 63 or the like, to cooling.

While various modifications may be made in the details of construction, as well as in the use and manufacture of the system and devices therefor, in accordance with this invention, it will be clear that this invention, both in process and in apparatus form, is of a broad nature, having application to the molding of lead alloy articles, as well as to the manufacture of battery grids, and also to metallic casting generally. For example, electric heating or other types of heating in lieu of any of the heating means 23, 31, 32 or 46 may be utilized, and dumping from the ladle 38 could also be controlled by the pyrometer 55 actuating the valve 42, instead of the device 60 performing such actuation. Thus the thermocouple 56 would sense when the ladle 38 should be pivoted, and initiate such pivoting. Accordingly, various modifications are all within the spirit and scope of the invention as recited in the appended claims.

What is claimed is:

1. A method of molding castings comprising the steps of initially providing a metallic casting material, then heating the casting material to a first temperature sufficient to allow liquid delivery thereof, less than the desired molding temperature, and below oxidation temperatures of said casting material, conveying the molten casting material to a heatable receptacle means and superheating the casting material to a second temperature above the first temperature and at least equivalent to the desired casting temperature of the material just prior to ladling of the material to a mold, and ladling the material at at least the desired casting temperature 55

into a mold.

2. The method of claim 1 wherein the method is specifically adapted for molding battery grid castings and the like, wherein at least a portion of the superheating step takes place in a controlled oxygen atmosphere for minimizing the formation of oxides on the surface of the molten metallic material.

3. The method of claim 1, wherein the superheating step takes place in a tubular device disposed in line between the location of initially heating the material and the ladling thereof, and wherein said superheating step comprises application of open flame to the tubular device.

4. The method of claim 1, wherein the superheating step comprises a first stage of heating the material just prior to delivery thereof to the ladle, to a temperature close to, but below a desired casting temperature of the material and a second stage of heating the material in a ladle, to at least the desired casting temperature of the material.

5. The method of claim 4, wherein the heating in the first stage comprises bringing the material to a temperature about 10° less than the desired casting temperature, at a location just prior to the location of heating in the ladle.

6. The method of claim 5, wherein the method is specifically adapted for molding battery grid castings and the like, wherein at least a portion of the superheating step takes place in a controlled oxygen atmosphere for minimizing the formation of oxides on the surface of the molten metallic material, wherein the superheating step takes place in a tubular device disposed in line between the location of initially heating the material and the ladling thereof, and wherein said superheating step comprises application of open flame to the tubular device.

7. The method of molding battery grids and the like of molten metal that includes at least lead material comprising the steps of first heating the material to a desired pumping temperature, just sufficient to allow pumping thereof, pumping the heated material to a superheater then superheating the material in a superheater of controlled oxygen atmosphere, to a temperature close to the desired casting temperature, delivering the superheated melt to a ladle, again heating the material in the ladle to at least a molding temperature, and pouring the material from the ladle into a mold.

8. The method of claim 7, including the steps of separately controlling the amount of heat applied to the material at the superheater and at the ladle.

9. The method of claim 1, wherein the superheating step includes superheating an amount greater than that needed for a given casting and returning the excess to the location of initial heating.

\* \* \* \* \*